

1

3,586,543

COATING TREATMENT OF METAL SURFACE  
Hiroshi Iijima, Yutaro Goto, and Masaji Terasaka, Kawasaki, Japan, assignors to Nippon Kakan Kabushiki Kaisha

No Drawing. Filed Oct. 16, 1968, Ser. No. 768,193  
Claims priority, application Japan, Oct. 20, 1967,

42/67,253

Int. Cl. C23f 15/60

U.S. Cl. 148—6.14

7 Claims

## ABSTRACT OF THE DISCLOSURE

Improved corrosion resistant films are formed on metal surfaces and coating properties are improved by immersing metals in solutions of molybdcic acid or salt thereof and a water soluble organic high polymer. The treatment is particularly effective for steel and galvanized steel sheets and pipes.

This invention relates to the coating treatment of metal surfaces, especially of steel and galvanized steel sheets and pipes, to improve the corrosion resistance and coating property by immersing the metals in a solution or emulsion containing molybdate thereof and a water-soluble organic high polymer, and then by heating the treated surface in order to form a film thereon.

It is well known in the prior art that chromic acid and phosphate treatments have been conducted in order to improve the corrosion resistance and coating property of steel sheets and galvanized steel sheets. However, conventional chromic acid and phosphate treatments have not been satisfactory with regard to corrosion resistance; the chromic acid treatment has been particularly unsatisfactory. Each of such treatments have resulted in inferior coating property. To obviate such deficiencies, various modifications have been proposed. Up to date, only unsatisfactory industrial results have been obtained.

It is accordingly a primary object of the present invention to obviate the above-mentioned difficulties and to provide a new method of forming a film having superior corrosion resistance and coating property on metals, especially on steel and galvanized steel sheets and tubes.

In accordance with the present invention, there is provided a method of coating a metal surface, which comprises immersing the metal in a solution or emulsion of molybdcic acid or salt thereof and water-soluble organic high polymer and then heating the metal.

The molybdenum-containing compound or compounds and the polymer or polymers cooperate to form an excellent insoluble film on the metal surfaces.

Molybdenum-containing compounds used herein include molybdcic acid or a salt thereof. Preferred salts are ammonium, sodium and calcium molybdate. Extremely small quantities of one or more of the acid and salts can be used. The solutions can contain from about 0.1 to about 30 percent by weight of such molybdenum compounds. Concentrations greater than about 0.5 mol of such compound in the solution of molybdenum compound and polymer are not advantageous.

The polymers of this invention are water-soluble organic polymers of high molecular weight, greater than about 10,000 (Viscosity Method). Such polymers include: acrylic, methacrylic, butadiene, styrene, maleic, linseed oil, polyvinyl alcohol, polyvinyl ether, alkyd, melamine-alkyd, melamine-formaldehyde and copolymers thereof. The concentration of resin in the treating solution ranges between about 0.05 and about 45 percent by weight.

When high level corrosion resistance is desired, the concentration of the treating solution is increased. The amount of coating on the metal surface is also increased.

2

With such increased concentrations and coatings, the heating or baking conditions are also varied in accordance with the type and amount of polymer used. Generally, higher baking temperatures are employed.

5 The treating solutions preferably contain an acid or salt thereof. Such additives can be used to adjust the pH of the solutions. Typical additives are mineral acids such as surfuric and phosphoric, organic acids such as acetic acid, acrylic acid, tartaric acid and citric acid, and salts such as sodium salt, potassium salt and calcium salt can be used.

10 Metal surfaces which have been immersed in the treating solutions are scorched or heated. Generally, they are subjected to temperatures of from about 200° C. to about 450° C. for intervals of from about 1/2 to about 2 minutes.

15 The invention is illustrated, and in no sense, limited by the following examples.

## EXAMPLE 1

20 A treating solution of 70 parts of a melamine alkyd resin 5% solution, 15 parts sodium molybdate 0.1 N solution, and 0.5 part of phosphoric acid 10% solution is used. A cold rolled steel sheet is immersed in the treating 25 solution, removed therefrom and passed through a neoprene rubber grooved roll for even distribution. It is then baked. The treated coated steel sheet has a yellowish, half-polish appearance. It was subjected to salt water spray (JIS) and outdoor exposure tests, the results 30 of which are about the same as those obtained in the same tests given to marketed steel sheets coated with electrolytic chromic acid. In a wetting test (49° C., 98% humidity), while marketed steel sheets coated by electrolytic chromic acid showed 50% of the area rusted after only 6 hours, 35 those treated with the method according to this invention showed the same degree of rust after 12 to 24 hours. As to the coating property of melamine alkyd and acrylic coating materials, the method used in the present invention showed the same degree of superior values as those given to cold rolled steel sheets in various tests applied on coated surfaces, in crosscut, bending, drawing, impact and Ericsen tests.

## EXAMPLE 2

40 45 Cold rolled steel sheet is immersed in a treating solution of 10 parts of magnesium molybdate of 0.1 N solution, and 70 parts of 7% melamine alkyd resin, the sheet is then taken out of the treating solution and is baked. Corrosion resistance and coating property are tested in the same manner as in Example 1 and similarly superior results have been obtained.

## EXAMPLE 3

50 55 Cold rolled steel sheet is immersed in a treating solution of 70 parts of 4/ alkyd (phthalic acid) resin solution, 15 parts of sodium molybdate 0.1 N solution and 1 part of 10% sulfuric acid. It is then taken out of the treating solution and is baked. Corrosion resistance and coating property have been tested in the same manner as in the case of Example 1 and the same superior results have been obtained.

## EXAMPLE 4

60 65 Cold rolled steel sheet is immersed in a treating solution of 10 parts of magnesium molybdate in 0.1 N solution and 70 parts of 5% alkyd resin (phthalic acid) solution. It is taken out of the treating solution and is then baked. A coating film of the same degree of superior corrosion resistance is obtained as in the case of Example 3. The film is rather soft, but its coating property is far superior to those in the case of cold rolled steel sheet which has not been so treated.

3  
EXAMPLE 5

Galvanized steel sheet is treated in a treating solution of 70 parts of 4% melamine alkyd resin solution, 5 parts of sodium molybdate of 0.1 N solution, and 0.3 part of 10% sulfuric acid. The sheet is removed from the treating solution and is passed through a roll. It is scorched by heat. The result of the wetting test (49° C., 98% humidity) with the treated sheet, indicated improvement in corrosion resistance toward white rust. Coating property when tested in the same manner as in the case of Example 1 turned out to be just as excellent as in the case of coatings given to cold rolled steel sheets by the method of this invention.

## EXAMPLE 6

Galvanized steel sheet is treated in a treating solution of 70 parts of 3% alkyd resin (phthalic acid) and 3 parts of magnesium molybdate of 0.1 N. The sheet is removed from the treating solution and is baked at 180° C. The treated sheet showed the same corrosion resistance toward white rust as the treated sheet of Example 5. The surface is soft, but the coating property is superior.

As has been discussed hereinabove, when the treatment according to this invention is applied to cold rolled steel sheet, it is possible to obtain a product with sufficient corrosion resistance required before being put to second process coating; and the same degree of superior coating

When this treatment is applied to galvanized steel sheets, the sheets have highly superior corrosion resistance toward white rust as compared with galvanized steel sheets subjected to a prior art chrome acid treatment. Further, galvanized steel sheets treated according to this invention have the same degree of superior coating property as in the case of cold rolled steel sheets.

Besides superior corrosion resistance and coating property, improvement in workability is to be expected. A superior effect in after-treatment of coated steel sheets other than galvanized steel sheets is also obtained.

Additional test results are provided in the following tables wherein:

Table I shows the results of JISZ 22371 salt water spray tests, that have been employed in Example 1. Steel sheets coated with 2 g./m.<sup>2</sup> of resin according to the method of this invention show a far more remarkable corrosion resistance than steel sheets treated by the electrolytic chromic acid and available in the market.

Table II shows results of wetting tests (49° C., 98% humidity). Galvanized steel sheets coated with 0.5 g./m.<sup>2</sup> resin according to the method of this invention show a far more excellent corrosion resistance against white rust than those treated by prior art chromic acid treatment.

TABLE I.—JIS SALT WATER SPRAY TEST<sup>1</sup>

| Test time (hours)                                                     | 1  | 3   | 5   | 8   |
|-----------------------------------------------------------------------|----|-----|-----|-----|
| Marketed steel sheet treated with electrolytic chromic acid:          |    |     |     |     |
| A                                                                     | 50 | 100 |     |     |
| B                                                                     | 10 | 50  | 100 |     |
| C                                                                     | 25 | 100 |     |     |
| Steel sheet treated according to this invention (examples 1, 2, 3, 4) | 10 | 25  | 50  | 100 |

<sup>1</sup> Values indicate percentage of rusted area.

TABLE II.—WETTING TEST<sup>1</sup>

| Test time (hours)                                                                                 | 1    | 2    | 5   | 10 | 24  |
|---------------------------------------------------------------------------------------------------|------|------|-----|----|-----|
| Galvanized steel sheet treated with chromic acid                                                  | 10   | 50   | 100 |    |     |
| Galvanized steel sheet treated with the method according to the present invention (examples 5, 6) | None | None | 10  | 50 | 100 |

<sup>1</sup> Values indicate percentage of rusted area.

## 4

Resin solutions employed in the Examples 1 to 6 are identified below for a better understanding of the invention.

5 Alyd (phthalic acid) resin is a denaturation of a phthalic alkyd resin being condensed with phthalic anhydride



and then denatured with linseed oil (oil content of about 50%-60%)

15 Melamine alkyd resin is a blending of denaturation of a melamine



which have been denatured with coconut oil and then condensed with said phthalic alkyd resin and coconut oil and then the melamine resin being condensed with said melamine and formaline (HCHO) is blended.

20 Melamine alkyd resin 5% solution used in the Example 1 is identified here as 5% aqueous solution of melamine alkyd resin. Two resins identified hereinabove have been used in the examples.

25 What is claimed is:

1. The method of coating a steel surface to improve the corrosion resistance and coating property thereof, which comprises:

30 immersing the steel in an aqueous solution containing from about 0.1 to about 30 percent by weight of molybdate acid or salt thereof and from about 0.05 to about 45 percent by weight of a water-soluble organic polymer having a molecular weight of greater than about 10,000 and heating the steel.

35 2. The method of claim 1 wherein the metal is galvanized steel.

40 3. The method of claim 1 wherein the salt is an ammonium, sodium or calcium molybdate.

45 4. The method of claim 1 wherein the polymer is selected from the group consisting of acrylic, methacrylic, butadiene, styrene, maleic acid, linseed oil, polyvinyl alcohol, polyvinyl ether, alkyd, melamine-alkyd, melamine-formaldehyde polymers and copolymers thereof.

50 5. The method of claim 1 wherein the solution contains a mineral acid or an organic acid to adjust the pH of said solution.

55 6. The method of claim 1, wherein the steel which has been so immersed is rolled before being heated.

7. The method of claim 1, wherein the steel is heated at a temperature of from about 200° C. to about 450° C.

## References Cited

## UNITED STATES PATENTS

|           |        |                 |          |
|-----------|--------|-----------------|----------|
| 3,052,575 | 9/1962 | Crane           | 148—6.14 |
| 3,175,964 | 3/1965 | Watanabe et al. | 148—6.2X |
| 3,185,596 | 5/1965 | Schiffman       | 148—6.2X |

60 65 RALPH S. KENDALL, Primary Examiner

C. WESTON, Assistant Examiner

U.S. Cl. X.R.

70 148—6.15; 117—132

UNITED STATES PATENT OFFICE  
CERTIFICATE OF CORRECTION

Patent No. 3,586,543 Dated June 22, 1971

Inventor(s) HIROSHI IIJIMA et al

It is certified that error appears in the above-identified patent and that said Letters Patent are hereby corrected as shown below:

Assignee is incorrectly identified - should be

Nippon Kokan Kabushiki Kaisha, as indicated in

Assignment recorded in Patent Office on October 16,  
1968 on Reel 2424 Frame 145.

Column 2, line 47 - delete "alyd" and replace with

---alkyd--- as indicated in specification, page 6,  
line 11.

Column 2, line 55 - delete "4/" and replace with

---4%--- as indicated in specification at page 6,  
line 17.

Column 3, lines 6-7 - delete "scorched by heat" and

replace with ---baked--- as indicated in amendment

filed September 23, 1970 at page 3 (re page 7, line 17  
of specification).

UNITED STATES PATENT OFFICE  
CERTIFICATE OF CORRECTION

Patent No. 3,586,543 Dated June 22, 1971  
Inventor(s) HIROSHI IIJIMA et al PAGE - 2

It is certified that error appears in the above-identified patent and that said Letters Patent are hereby corrected as shown below:

Column 3, line 27 - after "coating" (second occurrence)

insert ---property is obtained as in the case of cold  
rolled sheets.--- as indicated in specification at  
page 8, lines 16-17.

Signed and sealed this 2nd day of November 1971.

(SEAL)

Attest:

EDWARD M.FLETCHER, JR.  
Attesting Officer

ROBERT GOTTSCHALK  
Acting Commissioner of Patents